

## UNITED STATES PATENT OFFICE

2,314,810

## EXPLOSIVE COMPOSITION

Clarence Herman Winning, Woodbury, N. J., assignor to E. I. du Pont de Nemours & Company, Wilmington, Del., a corporation of Delaware

No Drawing. Application February 18, 1941,  
Serial No. 379,445

12 Claims. (Cl. 52—11)

This invention relates to explosive compositions containing a water-soluble inorganic salt, and more particularly to ammonium nitrate explosives.

This application is a continuation-in-part of my copending applications Serial No. 288,131, filed August 3, 1939, and Serial No. 354,825, filed August 30, 1940.

Ammonium nitrate is a very extensively used ingredient in present day high explosives of the dynamite type. It replaces nitroglycerine in increasingly larger proportions for a variety of reasons, particularly because it possesses high explosive strength, has outstanding safety properties, and is economically attractive. Ordinarily, it is used with some particular sensitizing agent, either explosive or non-explosive in nature. While ammonium nitrate explosives have been used with great success, one disadvantage of this ingredient has always been evident, namely, that it has a great affinity for water. Because of this fact, there is a tendency for explosive compositions high in ammonium nitrate to become hard and set on storage in the presence of even small amounts of moisture. This brings about a decreased sensitiveness of the explosive and a lesser degree of uniformity in performance. The water resistance of ammonium nitrate explosives is generally low because of the presence of this very soluble salt.

An object of the present invention is an explosive composition containing at least one water-soluble salt and having improved water resistance. A further object is an ammonium nitrate explosive of enhanced water resistance. A still further object is an explosive containing ammonium nitrate wherein an ingredient is present which tends to prevent the harmful penetration of water. Additional objects will be disclosed as the invention is described more at length hereinafter.

I have found that the foregoing objects are accomplished by including a grain sorghum derived from "Sorghum vulgare" as an ingredient in explosive compositions containing at least one water-soluble salt, said grain sorghum being capable of functioning in finely divided state as a protective agent against water for said soluble salt.

By the term "grain sorghum," as used above, I intend to designate various types of cereals such as kaffir corn and broom corn; in other words, cereals that may be classified botanically as "Andropogon sorghum." This will include any of certain grain sorghums derived from "Sorghum vulgare," having stout, short-jointed, semi-juicy stalks and erect heads. They are cultivated for grain and forage in various regions of the United States and in other countries. Broom corn and kaffir corn are the two representatives of this group best known and most common in the United States.

My invention is applicable with advantage to all explosive compositions containing a water-soluble salt, whether this salt is ammonium nitrate, sodium nitrate, a chlorate or perchlorate, or other soluble salt. I find it particularly important in the case of ammonium nitrate explosives, and especially in such compositions containing an explosive nitric ester, nitroglycerin for example. It should be understood, however, that the invention is applicable as well to explosive compositions which contain no ingredient which is itself an explosive, for example, compositions containing non-explosive sensitizing agents. Many compositions, for instance, contain ammonium nitrate or other oxidizing agent sensitized with materials such as aluminum or other finely divided metals. Likewise, certain ammonium nitrate explosives are sensitized with various forms of carbon, and explosive and non-explosive nitrated hydrocarbons, for example paraffin, charcoal, dinitro-toluene, and the like. My invention is equally applicable to these compositions, since they contain the water-soluble salt which must be protected from wet conditions in the field.

The advantages of my invention are illustrated by the following specific embodiments, in which A and B represent ammonia dynamites of similar compositions, A containing ordinary carbonaceous combustibles while B contains ground kaffir corn:

|                              | A            | B     |
|------------------------------|--------------|-------|
| Nitroglycerin.....           | percent..... | 14.0  |
| Ammonium nitrate.....        | do.....      | 36.5  |
| Calcium stearate.....        | do.....      | 0.3   |
| Sodium nitrate.....          | do.....      | 35.8  |
| Wood pulp.....               | do.....      | 1.0   |
| Prior art meals.....         | do.....      | 8.9   |
| Kaffir corn.....             | do.....      | 8.0   |
| Sulfur.....                  | do.....      | 3.0   |
| Chalk.....                   | do.....      | 0.5   |
|                              | 100.0        | 100.0 |
| Density—ctgs./50lbs.—1½ x 8" | 112          | 109   |

The protection afforded the explosive by the ground kaffir corn in sample B, was demonstrated by the results of a leaching test. Using 1¼ x 8" cartridges of compositions A and B, these were partly opened and immersed in 1½ x 9" cans, filled with water. The supernatant liquid in the two cases after 24 hours amounted to 125 and 140 cc., respectively, for A and B, the respective specific gravities of said liquids being 1.140 and 1.025, showing the greater protection from loss of soluble salts in the case of the explosive containing the kaffir corn. The lesser degree of wetness of the same powder is shown by the fact that A, after the leaching test, comprised 5¾" of highly wet powder, 1¼" of moderately wet powder, and no slightly damp powder against cor-

responding quantities of 1", 3½", and 2½" for B.

In a second leaching test, additional evidence was given of the improved resistance to water imparted by the presence of the kaffir corn. Cartridges of 4" x 10" dimensions were used, and four holes of ¾" diameter were made in the side wall at each end, the cartridges then being subjected to a water pressure of 15 lbs. per square inch for 24 hours. At the end of the test, dynamite A, containing meals of the prior art, had shrunk to a column of highly wet material of 3 x 6½" size. The weight of the cartridge had decreased from 2622 to 1563 grams, some of the latter weight being due to the water present. In the case of dynamite B, containing kaffir corn, the weight of the cartridge had increased from 2680 to 2831 grams. Of the 4" diameter column of powder remaining, 2" was high wet, 2" slightly damp, and 4" entirely dry. The explosive B was capable of detonation by a blasting cap at the end of the test.

The kaffir corn, when present in explosives of the type described, is capable of forming a cohesive and protective paste with the more or less dilute solutions produced when water comes in contact with the outer or exposed portions of explosives containing water-soluble salts. Ordinary flours, meals, and starches do not disperse satisfactorily and do not form protective pastes. As examples of these latter materials, I may mention untreated wheat flour, corn meal, tapioca starch, and the like.

The dispersions formed by mixture of ordinary starch products with relatively small amounts of either water or dilute nitrate solutions, without application of heat, are such that there is a rapid separation of the flour, meal, starch, or the like. The ground kaffir corn acts differently in that the greater part of the material remains colloidally dispersed and suspended, on dilution of a relatively dry paste with dilute nitrate solution, even though no heat has been applied at any time.

When kaffir corn meal according to my invention is used in compositions such as ammonia dynamites, it appears that the entrance of the first traces of water brings about a paste or gel formation. This gelatinization in the outer portion of the explosive retards the rate of water penetration toward the interior of the explosive column. The gelatinous structure formed also prevents segregation of liquid or solid ingredients of the explosive such as would be caused by water penetration and softening of the composition. The cohesive gel or paste also decreases the loss of solid or liquid ingredients from partly opened cartridges by reason of gravity flow. The leaching of soluble salts is likewise lessened by the presence of the paste.

It will be understood that, in order to obtain the most favorable results, the kaffir corn or broom corn meal, or similar meal, should be in finely divided condition. Preferably, said meal should be in a state of subdivision such that the major portion, that is more than 50%, will pass a 60-mesh screen. Furthermore, the ground kaffir corn is desirably included in the explosive composition in pulverulent form during the manufacture of the explosive composition, no paste being formed at that time. I do not intend to be limited to meal of this degree of fineness, however. Likewise, I may wish to introduce into the explosive composition a small amount of a

water-insoluble metal soap, such as calcium stearate, which will have a protective and coating effect on the ammonium nitrate against water or moisture. The presence of this latter ingredient, together with the kaffir corn meal, gives very beneficial results. The ground kaffir corn is effective, however, without the presence of the water-insoluble soap. Preferably, said kaffir corn meal will be used in an amount not greater than 15%, and I find a quantity between 1 and 9% to be advantageous.

The invention is applicable with great advantage in ammonia dynamites containing ammonium nitrate and nitroglycerin in amounts not exceeding 25%, for example between 3 and 25%. It has important applications also in the case of compositions containing other high explosive compounds, such as nitrostarch, trinitrotoluene, and the like, in the presence of ammonium nitrate or other water-soluble salt. Furthermore, it is effective in the case of compositions in which the ammonium nitrate is sensitized by means of paraffin, dinitrotoluene, carbon, aluminum, other powdered metals and alloys, and many other materials.

The ground grain sorghum such as kaffir corn or broom corn, according to my invention, has been stated to be present preferably in pulverulent form during the manufacture of the explosive, since in this form the meal or flour functions in the peculiarly effective manner desired in protecting the explosive against water penetration.

My invention has been described in detail in the foregoing. It will be apparent, however, that many variations may be introduced in methods of application or in compositions without departure from the scope of the invention. I intend to be limited, therefore, only by the following patent claims.

I claim:

1. An explosive composition comprising a water-soluble oxygen-supplying inorganic salt, a sensitizing agent, and a cereal meal of the species *Andropogon sorghum* in pulverulent form.

2. The explosive composition of claim 1, in which the cereal meal is kaffir corn.

3. The explosive composition of claim 1, in which the cereal meal is broom corn.

4. An explosive composition comprising ammonium nitrate, a sensitizing agent, and a cereal meal of the species *Andropogon sorghum* in pulverulent form.

5. The explosive composition of claim 4, in which the cereal meal is kaffir corn.

6. The explosive composition of claim 4, in which the cereal meal is broom corn.

7. An explosive composition comprising ammonium nitrate, an explosive sensitizing agent, and kaffir corn meal in pulverulent form.

8. The explosive composition of claim 7, wherein the sensitizing agent is nitroglycerin.

9. The explosive composition of claim 7, wherein the sensitizing agent is an aromatic nitrocompound.

10. An explosive composition comprising ammonium nitrate, a non-explosive sensitizing agent and kaffir corn meal in pulverulent form.

11. The explosive composition of claim 10, in which the sensitizing agent is a powdered metal.

12. An explosive composition comprising ammonium nitrate, between 3 and 25% of nitroglycerin, and not more than 15% of kaffir corn meal in pulverulent form.